

## UNITED STATES PATENT OFFICE

GEORGE HOLLAND ELLIS, OF SPONDON, NEAR DERBY, ENGLAND, ASSIGNEE TO  
CELANESE CORPORATION OF AMERICA, A CORPORATION OF DELAWARE

## DYEING OR COLORATION OF CELLULOSE ACETATE

No Drawing. Application filed April 6, 1926, Serial No. 100,178, and in Great Britain May 2, 1925.

This invention relates to the dyeing of cellulose acetate in the form of yarns, threads, fabrics, films or other goods consisting of or containing it, by processes involving the oxidation of aniline, para-amino phenol, para-phenylenediamine, benzidine, tolidine, para-amino diphenylamine, alpha-naphthylamine, or other amino bodies on the fibre or material.

10 It has been proposed to dye cellulose acetate by processes involving the oxidation of amino bodies on the fibre, by the following methods:—

15 1. The "single bath" process, in which the goods are treated in a bath containing the amino base or salt thereof, together with oxidizing agents e. g. bichromates.

20 2. The "two bath" process, in which the goods are first soaked in a solution of the amino body or of a salt thereof, the oxidation being effected in a separate bath containing persulphates, perborates and the like, or the oxidation being effected in the exhausted base-bath after addition thereto of persulphates, perborates and the like. The presence in the baths of acids, salts and protective colloids has also been proposed for this "two bath" process.

25 3. The "ageing" process, in which the goods are first treated with a solution of the amino body or of a salt thereof, together with oxidizing agents and catalysts, the goods being dried after soaking, and then heated in a warm atmosphere to effect or to complete oxidation. The presence in the impregnation bath of salts, acids and protective colloids has also been proposed.

30 The dyeings produced on cellulose acetate by the oxidation of amino bodies on the fibre by methods hitherto proposed have not been satisfactory, and in nearly all cases the processes cause loss of lustre of the fibre and yield dyeings loose to rubbing. In the "single bath" process above referred to there is usually formation in the bath of insoluble coloring matter, which is adsorbed on the surface of the goods, causing loss of lustre and looseness to rubbing. In the "two bath" process there is a great tendency during oxidation for the amino body to be withdrawn from the

fibre to the bath, and the dyeings produced suffer from the same defects as those produced by the "single bath" process. In the "ageing" process a considerable amount of surface pigmentation of the goods results 55 and the method yields dyeings loose to rubbing, with loss of lustre of the fibre.

It has now been found that if the amino body or bodies are applied to the cellulose acetate from aqueous solutions or dispersions 60 so that the fibre gradually absorbs the base or bases in the manner in which it absorbs dyestuffs from aqueous solutions or dispersions; and if then, preferably after rinsing, solutions of suitable oxidizing agents,—with 65 or without addition of catalysts or of salts, or of both,—are mechanically applied by impregnation, and then, without rinsing, but preferably after drying, the goods are "aged" in an atmosphere of warm, moist air or of 70 steam or air and steam, oxidation proceeds exceedingly well, and the results are free from the defect of looseness to rubbing and loss of lustre of the fibre.

According to the invention the amino body 75 or bodies are applied on the fibre or material from aqueous solutions or dispersions, and subsequently, preferably after rinsing, the goods are impregnated with a solution or solutions of suitable oxidizing agents; containing or not containing catalysts or salts, or both catalysts and salts, and thereafter the goods, without rinsing, but preferably after drying, are subjected to "ageing" in an atmosphere of warm moist air, or of steam, or 80 air and steam.

The amino body or bodies may be applied to the goods in any suitable dilution, in form of their water soluble salts, e. g. hydrochlorides.

90 Or the amino body or bodies may be applied to the goods in any suitable dilution, in form of their soluble or more soluble modifications prepared by treating them with sulphuricinoleic acid or other sulphated fatty 95 acids or other bodies of oily or fatty characteristics, namely higher fatty acids or sulphonated or other derivatives thereof containing salt forming groups capable of forming soluble salts with alkalies or ammonia, 100

or with salts of such bodies, such for instance as their alkali or ammonium salts; that is to say by treating the amino body or bodies with the solubilizing agents of the character referred to in British specification No. 5 219,349 and the corresponding U. S. Patent No. 1,618,413. For simplicity, all of said solubilizing agents (including the salts) are hereinafter and in the claims included in the term body of oily or fatty characteristics. Corresponding to what is stated in the said specifications, the soluble or more soluble modifications of the amino body or bodies may be prepared by stirring up or 10 treating the amino body or bodies with one or more of the said solubilizing agents, heating if necessary, and the mass can be afterwards diluted with water or aqueous alkali filtered if required, and added to 15 the dyebaths. "Solid" solutions or concentrated preparations of the amino body or bodies may be made by heating them with the body or bodies of oily or fatty characteristics, for instance oleic, stearic, palmitic, or 20 sulphorcinoleic acid, etc., (or their salts) either by treatment in presence of little or no water, or by treatment in presence of larger quantities of water with subsequent concentration or drying. The "solid" solutions or concentrated solubilized preparations may 25 be diluted with hot water and added to the dyebath.

Or again, the amino body or bodies may be applied in the form of their soluble or more soluble modifications prepared by the methods described in prior United States Patents Nos. 1,618,414 granted February 22, 1927, 30 1,690,481 granted November 6, 1928, and 1,694,413 granted December 11, 1928.

As stated in the said U. S. Patent No. 1,618,414 the method therein indicated consists in a pretreatment with one or more carbocyclic solubilizing agents, that is to say carbocyclic compounds containing in their 40 structure one or more salt-forming groups or with sodium or other salts of said compounds, or with mixtures of such carbocyclic solubilizing agents, or mixtures of one or more thereof with one or more of the aforesaid bodies of oily or fatty characteristics; as instances of such carbocyclic solubilizing agents the U. S. Patent No. 1,618,414 mentions naphthenic acids, naphthene sulphonic acids, or other carboxylic acids or sulphonic 45 acids of cycloparaffins; phenols; sulphonic acids, carboxylic acids, phenol sulphonic acids or other derivatives of the benzene, naphthalene or anthracene series; or other derivatives of saturated or non-saturated 50 cyclic hydrocarbons containing one or more salt forming groups; or sodium or other salts of any of such compounds. The solubilization of the amino body or bodies with the solubilizing agents or solubilizing mixtures 55 referred to in the said U. S. Patent No. 60

1,618,414 may be effected similarly to the solubilization with aforesaid bodies of oily or fatty characteristics, and the solubilized forms or modifications may be similarly applied to the goods.

The method indicated in U. S. Patent No. 1,694,413 consists in a pretreatment with solubilizing agents consisting of or comprising one or more Twitchell reagents, which term includes sulpho-aromatic fatty acids such as sulphobenzene stearic acid, sulphophenol stearic acid or sulphonaphthalene stearic acid, and salts of sulpho-aromatic fatty acids. The solubilization of the amino body or bodies with the solubilizing agents referred to in U. S. Patent No. 1,694,413 may be effected similarly to the solubilization with the aforesaid bodies of oily or fatty characteristics, and the solubilized forms or modifications may be similarly applied to the goods.

The method indicated in U. S. Patent No. 1,690,481 consists in a treatment comprising the employment, in conjunction with the aforesaid bodies of oily or fatty characteristics, of auxiliary solvents, and the said U. S. Patent No. 1,690,481 gives as examples of such auxiliary solvents:—alkyl or alkylene halides such for instance as tetrachlorethane, trichloreethylene; simple or "mixed" derivatives of the cyclic or aromatic series containing one or more amino, chlor or hydroxy groups, such for example as cresols, alkylanilines, toluidines, chlorphenols, mono- or poly-chlor benzenes; hydrogenated derivatives of such or other aromatic compounds, such for example as hexahydrophenol, hexahydrocresols, hexahydrobenzene, dekahydronaphthalene, tetrahydronaphthalene and the like. Corresponding to what is stated in the said U. S. application Serial No. 48,666, which has issued as U. S. Patent No. 1,690,481 the amino body or bodies may be treated with one or more of the aforesaid bodies of oily or fatty characteristics and one or more of the auxiliary solvents,—either in any order separately, or together in admixture,—at any suitable temperature or pressure, in presence or absence of water, and the solubilized modifications so obtained may be added to the dyebaths. It will be understood that where the amino body or bodies are solubilized in accordance with the method described in U. S. application Serial No. 48,666 for the purpose of practising the present invention, the auxiliary solvent or solvents employed will be of a nature suitable to the process of the present invention, and that in such cases the use as auxiliary solvents of alkylanilines or other amino bodies or phenolic or naphthoic or other bodies which would be absorbed substantively by the cellulose acetate and enter into oxidation reactions, would be avoided.

The solutions or colloidal dispersions of the amino body or bodies may be applied to

the goods in any suitable manner such as are employed in ordinary dyeing practice. Suitable dyeing machinery may, if desired be employed, for instance the ordinary reel or winch machine for knitted goods, or the revolving roller machine for hanks. As before mentioned the goods are preferably rinsed after the application of the amino body or bodies and prior to the impregnation with the oxidizing liquor.

- 10 The mechanical impregnation of the solutions containing the oxidizing agents may be performed in any suitable way, for instance in a "padding" or other mangle which gives a good squeeze out of excess liquor; or the goods, especially hanks, may be wrung out on sticks by hand after dipping; the impregnation liquor is preferably applied to the goods in the cold.
- 15 As oxidizing agents I may employ chlorates (such as sodium or potassium chlorates), hypochlorites, bichromates and the like, and catalysts which I have found useful are salts of vanadium, iron or copper, but any 20 other suitable catalyst may be employed. As salts other than catalysts, I may employ any suitable soluble salts, as for instance, Glauber salt, ammonium chloride, barium chloride, calcium chloride, magnesium chloride and 25 the like. Where acid salts likely to cause 30 tendering of the fibre are used, acetates such as calcium acetate or sodium acetate may be added to the impregnation liquor. As before mentioned the goods are preferably dried 35 without rinsing after the impregnation.

The "ageing" treatment in an atmosphere of warm, moist air, steam, or air and steam may be carried out at any suitable temperature and for any suitable length of time, the 40 treatment varying with the results desired and the amino body or bodies employed. The "ageing" treatment may be performed in any suitable apparatus, as for instance in the continuous type of "ageing" machine which 45 permits variable conditions of atmosphere, or in the simple "box" steamer or "ager". After "ageing" the goods may be rinsed, soaped, or otherwise treated to remove the metallic salts and finished as desired.

- 50 By the process of the present invention it is possible to obtain a great variety of shades according to the amino body or bodies employed. By way of example the following shades may be obtained on acetyl cellulose 55 when using the following amino bodies for the process:

|                         |                 |
|-------------------------|-----------------|
| Aniline                 | Grey or black.  |
| Para aminophenol        | Fawn-brown.     |
| Paraphenylenediamine    | Rich red-brown. |
| Para aminodiphenylamine | Black.          |
| Tolidine                | Green-black.    |
| Alphanaphthylamine      | Dull brown.     |

It is to be understood that I do not limit 65 myself to these examples, as a very great

number of amino bodies may be used and a great variety of shades may be obtained.

The following are some examples of the manner in which the invention may be performed, it being understood that these are given only by way of illustration and can be varied widely without departing from the invention.

#### Example I

To dye 10 lbs. of cellulose acetate yarn in hank form a full deep black,  $\frac{3}{4}$  lb. of para aminodiphenylamine base are intimately mixed with 6 lbs., of 50% Turkey red oil diluted with soft water, and heated to  $80^{\circ}$  C. for a short while to effect solubilization or dispersion. This is then diluted with hot water and added through a filter cloth to a dyebath containing 25 gallons of soft water at  $80^{\circ}$  C. The goods are now entered at this temperature and worked for two hours. After rinsing well in soft water they are impregnated cold with their own weight of an oxidation solution of the following composition:

2 parts of gum tragacanth dissolved in 300 parts of water.  
8 parts of chromium chloride in 56 parts of water.  
4 parts of aluminium chloride in 50 parts of water.  
3 parts of cupric chloride in 50 parts of water.  
60 parts of sodium chlorate in 120 parts of water.

Add water to make up to a total of 1000 parts.

The goods are now "aged", (preferably after drying at a moderate temperature), for 5 minutes in a steam "ager", washed off in hot water, or very dilute (1 cc. per litre) formic acid to remove mineral matter. The yarn has now acquired a dead black coloration, lustre and handle being unimpaired. It may now be dried and finished as desired.

#### Example II

To dye 10 lbs. of cellulose acetate in hank form a medium brown shade,  $\frac{1}{2}$  lb. of benzidine is solubilized or dispersed by warming with  $2\frac{1}{2}$  lbs. of the dispersing agent prepared by sulphonating a mixture of naphthalene and oleic acid (Twitchell reagent). The solubilized modification or dispersion thus obtained is diluted with boiling soft water, and added through a filter cloth to a dyebath containing 25 gallons of soft water. The goods are now entered, raised to  $70-75^{\circ}$  C. in  $\frac{3}{4}$  hour and worked at this temperature for 1 hour; they are now lifted and rinsed, and the base is oxidized by the impregnation and "ageing" process as detailed in the previous example.

After rinsing in dilute formic acid the goods will have acquired a dull brown shade,

the lustre and handle being unimpaired. They are now ready for drying or otherwise treating as desired.

*Example III*

5 To dye 10 lbs. of cellulose acetate in hank form a fawn-brown shade,  $\frac{1}{2}$  lb. of para aminophenol is dissolved in 25 gallons of water, the goods are added, and the temperature is raised to 70-75° C. in  $\frac{3}{4}$  hour, being maintained a further  $\frac{3}{4}$  hour at this temperature. After lifting and rinsing, the base is oxidized as in Example I by the impregnation and "ageing" method. They will have 10 acquired a fawn-brown color, lustre and handle being unimpaired. After rinsing in 15 1 gram per litre of formic acid solution, the goods are now ready for drying or otherwise treating as desired.

20 *Example IV*

To dye 10 lbs. of cellulose acetate yarn in hank form a deep brown shade,  $\frac{1}{2}$  lb. of paraphenylenediamine is dissolved in sufficient water and added to a dyebath containing 25 25 25 gallons of water. The goods are entered, and the temperature is raised to 70°-75° C. in  $\frac{3}{4}$  hour and maintained at this temperature for one hour. After rinsing, the 30 goods are impregnated with a solution made up as follows:—

2 parts of gum tragacanth in 300 parts of water.  
35 4 parts of aluminium chloride in 50 parts of water.  
3 parts of cupric chloride in 50 parts of water.  
150 parts of sodium bichromate in 100 parts of water.  
40 Make up to 1000 parts with water.

After squeezing evenly so that the fibre contains only its own weight of oxidizing mixture, the goods are aged for 5 minutes in a 45 steam ager and rinsed in very dilute formic acid. They may now be dried and finished as desired.

What I claim and desire to secure by Letters Patent is:—

- 50 1. Process for dyeing materials containing cellulose acetate, comprising applying to the materials at least one amino body from an aqueous solution, mechanically impregnating with a solution comprising an oxidizing agent and thereafter, without rinsing, subjecting to aging in a warm moist atmosphere.  
55 2. Process for dyeing materials containing cellulose acetate, comprising applying to the materials at least one amino body from an aqueous colloidal solution, mechanically impregnating with a solution comprising an oxidizing agent and thereafter, without rinsing, subjecting to aging in a warm moist atmosphere.  
60 65 3. Process for dyeing materials containing

cellulose acetate, comprising applying to the materials at least one amino body from an aqueous colloidal solution prepared by pre-treating the amino body with a solubilizing agent, mechanically impregnating with a solution comprising an oxidizing agent and thereafter, without rinsing, subjecting to aging in a warm moist atmosphere. 70

4. Process for dyeing materials containing cellulose acetate, comprising applying to the materials at least one amino body from an aqueous colloidal solution prepared by pre-treating the amino body with a solubilizing agent comprising a body of oily or fatty characteristics, mechanically impregnating with a solution comprising an oxidizing agent and thereafter, without rinsing, subjecting to aging in a warm moist atmosphere. 75

5. Process for dyeing materials containing cellulose acetate, comprising applying to the materials at least one amino body from an aqueous solution, rinsing, mechanically impregnating with a solution comprising an oxidizing agent and thereafter, without rinsing, drying and subjecting to aging in a warm moist atmosphere. 85

6. Process for dyeing materials containing cellulose acetate, comprising applying to the materials at least one amino body with an aqueous colloidal solution, rinsing, mechanically impregnating with a solution comprising an oxidizing agent and thereafter, without rinsing, drying and subjecting to aging in a warm moist atmosphere. 95

7. Process for dyeing materials containing cellulose acetate, comprising applying to the materials at least one amino body from an aqueous solution, mechanically impregnating with a solution comprising an oxidizing salt and thereafter, without rinsing, subjecting to aging in a warm moist atmosphere. 100

8. Process for dyeing materials containing cellulose acetate, comprising applying to the materials at least one amino body from an aqueous colloidal solution, mechanically impregnating with a solution comprising an oxidizing salt and thereafter, without rinsing, subjecting to aging in a warm moist atmosphere. 110

9. Process for dyeing materials containing cellulose acetate, comprising applying to the materials at least one amino body from an aqueous solution, mechanically impregnating with a solution comprising an oxidizing agent and a catalyst and thereafter, without rinsing, subjecting to aging in a warm moist atmosphere. 115

10. Process for dyeing materials containing cellulose acetate, comprising applying to the materials at least one amino body from an aqueous colloidal solution, mechanically impregnating with a solution comprising an oxidizing agent and a catalyst and thereafter, without rinsing, subjecting to aging in a warm moist atmosphere. 125

11. Process for dyeing materials containing cellulose acetate, comprising applying to the materials at least one amino body from an aqueous solution, mechanically impregnating with a solution comprising an oxidizing agent and thereafter, without rinsing, subjecting to aging by steaming. 70
12. Process for dyeing materials containing cellulose acetate, comprising applying to the materials at least one amino body from an aqueous colloidal solution, mechanically impregnating with a solution comprising an oxidizing agent and thereafter, without rinsing, subjecting to aging by steaming. 75
13. Process of dyeing materials containing cellulose acetate which comprises applying to such materials an aqueous solution of at least one amino compound, subjecting the thus treated material to the action of oxidizing agents, and thereafter, aging the said material in a warm, moist atmosphere. 80
14. Process of dyeing materials containing cellulose acetate which comprises applying to such materials an aqueous solution of at least one amino compound prepared by pretreating the amino body with a solubilizing agent comprising a body of oily or fatty characteristics, mechanically impregnating the thus treated material with a solution containing a chlorate, and thereafter, without rinsing, subjecting it to aging in a warm, moist atmosphere. 85
15. Process of dyeing materials containing cellulose acetate which comprises applying to such materials an aqueous solution of at least one amino compound prepared by pretreating the amino body with a solubilizing agent, rinsing, mechanically impregnating the thus treated material with a solution containing a chlorate, and thereafter, without rinsing, subjecting the material to aging in a warm, moist atmosphere. 90
16. Process of dyeing materials containing cellulose acetate which comprises applying to such materials an aqueous solution of at least one amino compound prepared by pretreating the amino body with a solubilizing agent, rinsing, mechanically impregnating the thus treated material with a solution containing a chlorate, and thereafter, without rinsing, drying, and subjecting the material to aging in a warm, moist atmosphere. 95
17. Process of dyeing materials containing cellulose acetate which comprises applying to such materials an aqueous solution of at least one amino compound, mechanically impregnating the thus treated material with a solution containing a chlorate and a catalyst, and thereafter, without rinsing, drying, and subjecting it to aging in a warm, moist atmosphere. 100
18. Process of dyeing materials containing cellulose acetate which comprises applying to such materials an aqueous solution of at least one amino compound, mechanically im- 105
- pregnating the thus treated material with a solution containing a chlorate and a copper salt, and thereafter, without rinsing, drying, and subjecting it to aging in a warm, moist atmosphere. 110
19. Process of dyeing materials containing cellulose acetate which comprises treating such material in a bath at 80° C. containing para-amino diphenyl-amine base intimately mixed with Turkey red oil and soft water, rinsing the material, mechanically impregnating it with a water solution containing a gum, chromium chloride, aluminum chloride, cupric chloride and sodium chlorate, drying the material and then aging it in a damp, moist atmosphere. 115
- In testimony whereof I have hereunto subscribed my name.
- GEORGE HOLLAND ELLIS. 120
- 130